



US008283288B2

(12) **United States Patent**  
**Shinohara et al.**

(10) **Patent No.:** **US 8,283,288 B2**  
(45) **Date of Patent:** **Oct. 9, 2012**

(54) **THERMAL TRANSFER RECEIVING SHEET**

(75) Inventors: **Hideaki Shinohara**, Tokyo (JP); **Yoshihiro Shimizu**, Tokyo (JP); **Yoshio Mizuhara**, Tokyo (JP); **Mitsuru Tsunoda**, Tokyo (JP)

(73) Assignee: **Oji Paper Co., Ltd.**, Tokyo (JP)

(\*) Notice: Subject to any disclaimer, the term of this patent is extended or adjusted under 35 U.S.C. 154(b) by 905 days.

(21) Appl. No.: **11/795,146**

(22) PCT Filed: **Jan. 20, 2006**

(86) PCT No.: **PCT/JP2006/301255**

§ 371 (c)(1),  
(2), (4) Date: **Jul. 12, 2007**

(87) PCT Pub. No.: **WO2006/080410**

PCT Pub. Date: **Aug. 3, 2006**

(65) **Prior Publication Data**

US 2008/0008896 A1 Jan. 10, 2008

(30) **Foreign Application Priority Data**

Jan. 28, 2005 (JP) ..... 2005-021368

(51) **Int. Cl.**

**B41M 5/035** (2006.01)  
**B41M 5/50** (2006.01)

(52) **U.S. Cl.** ..... **503/227; 8/471**

(58) **Field of Classification Search** ..... None  
See application file for complete search history.

(56) **References Cited**

**U.S. PATENT DOCUMENTS**

|                 |   |         |               |       |           |
|-----------------|---|---------|---------------|-------|-----------|
| 5,011,814 A     | * | 4/1991  | Harrison      | ..... | 503/227   |
| 5,837,649 A     |   | 11/1998 | Nozaki        | ..... | 503/227   |
| 2004/0067345 A1 |   | 4/2004  | Hladik et al. | ..... | 428/195.1 |
| 2004/0247804 A1 |   | 12/2004 | Kim et al.    | ..... | 428/32.36 |

**FOREIGN PATENT DOCUMENTS**

|    |             |         |
|----|-------------|---------|
| EP | 1 095 784   | 5/2001  |
| EP | 1 241 017   | 9/2002  |
| EP | 1 457 353   | 9/2004  |
| EP | 1 481 812   | 12/2004 |
| JP | 5-92669     | 4/1993  |
| JP | 6-239036    | 8/1994  |
| JP | 10-29379    | 2/1998  |
| JP | 2002-337463 | 11/2002 |
| JP | 2003-191652 | 7/2003  |
| JP | 2005-313595 | 11/2005 |

**OTHER PUBLICATIONS**

European Search Report mailed Jan. 30, 2008 (6 pages).

\* cited by examiner

*Primary Examiner* — Bruce H Hess

(74) *Attorney, Agent, or Firm* — Kratz, Quintos & Hanson, LLP

(57) **ABSTRACT**

The present invention provides a thermal transfer receiving sheet comprising a sheet-like support, an image receiving layer containing, as a main component, a dye-dyeable resin formed on one surface of the sheet-like support, and a back surface coating layer containing an adhesive resin formed on the other surface of the sheet-like support, wherein the back surface coating layer contains a polyvinyl pyrrolidone resin in an amount of 1 to 50% by weight based on the total solid content of the back surface coating layer.

**5 Claims, No Drawings**

## THERMAL TRANSFER RECEIVING SHEET

## TECHNICAL FIELD

The present invention relates to a thermal transfer receiving sheet (hereinafter referred simply to as a receiving sheet). More particularly, the present invention relates to a receiving sheet which has good printability in an ink jet printer required for a back surface coating layer (hereinafter simply referred to as a back surface layer) of a receiving sheet, and also comprises a back surface layer having sufficient writability for various writing instruments.

## BACKGROUND ART

A high image quality color hard copy printing system using a dye thermal transfer system is composed of a printer, a thermal transfer sheet (hereinafter simply referred to as an ink ribbon) and a receiving sheet. As a general method for forming a color image on the receiving sheet, the ink ribbon having color material layers composed of three or four colors i.e. yellow, magenta, cyan and, if necessary, black, is closely contacted with the receiving sheet, which is provided with an image receiving layer (hereinafter, simply referred to as receiving layer), and they are transported through a heating device and pressed by constant pressure from a platen roller. Then, heat generating part of the heating device is selectively made to generate heat, and the dye contained in the color material layers of the ink ribbon is transported to the receiving layer of the receiving sheet to obtain an image. An ink ribbon comprises color material layers consisting of three or four different colored-layers stacked on each other. A color image is formed by sequentially transferring each color, three or four times for each, at the same position of the receiving sheet, thereby superposing each color on the same position. In such a printer of a dye thermal transfer system, the receiving sheet is usually supplied in a sheet state.

Generally, the receiving sheet is formed of a sheet-like support, with a receiving layer formed on one surface thereof, having an excellent dyeing property with dye transferred from an ink ribbon, and a back surface layer formed on the other surface, and provides various properties such as printability in an ink jet printer and writability with various writing instruments.

In the receiving sheet, writing is occasionally performed on the surface (back surface side) opposite the surface of the receiving layer on which an image is formed. It is necessary that writing can be performed by various writing instruments. Recently, printability by an ink jet printer is also required. When the support is a synthetic paper or a plastic film, the support is insufficient in printability in an ink jet printer and is also insufficient in writability for various writing instruments. In order for the back surface layer to have excellent writability, it is necessary that the back surface layer exhibits sufficient writability for oily- or water-based pen-type writing instruments, pencils or the like. Moreover, good printability is also required for printing by a printer, such as an ink jet printer.

As a back surface layer of the thermal transfer receiving paper, some proposals have been made for the purpose of providing writability for various writing materials. In order to improve writability, the back surface layer containing an inorganic pigment includes, for example, a back surface layer containing plate-like barium sulfate (see, for example, Japanese Unexamined Patent Publication (Kokai) No. 9-24676 (page 2)), a back surface layer containing silica microparticles having a specific particle size (see, for example, Japa-

nese Unexamined Patent Publication (Kokai) No. 3-180393 (page 1)), and a back surface layer containing microsilica and acetyl cellulose (see, for example, Japanese Unexamined Patent Publication (Kokai) No. 8-244362 (page 2)).

However, in the back surface layer containing these inorganic pigments, since the inorganic pigments are generally hard, there is a problem that the ink receiving layer may be damaged because the surface of the ink receiving layer is rubbed with the back surface layer when the ink receiving sheet travels through a thermal transfer printer, resulting in poor printing quality. Moreover, printability and drying in an ink jet printer are also insufficient and an improvement is required.

In order to solve the above problem, a back surface layer with low hardness, containing an organic pigment, has also been proposed. For example, there is a back surface layer containing spherical silicone microparticles (see, for example, Japanese Unexamined Patent Publication (Kokai) No. 7-108775 (page 2)), a back surface layer containing cellulose microparticles (see, for example, Japanese Unexamined Patent Publication (Kokai) No. 5-92669 (page 2)), a back surface layer containing organic and/or inorganic particles, a higher aliphatic salt, and a binder as main components (see, for example, Japanese Unexamined Patent Publication (Kokai) No. 1-241491 (Page 1)), and a back surface layer containing particles of a Mohs hardness of 1 to 4 (see, for example, Japanese Unexamined Patent Publication (Kokai) No. 6-239036 (Page 2)). However, in the back surface layer containing an organic pigment, because of slight damage to the receiving layer by the back surface layer, pencil writability is insufficient, and also printability and drying in an ink jet printer are also insufficient.

A proposal to improve writability by mixing inorganic or organic pigment with the back surface layer improves writability by conventional writing instruments such as water- and oil-based pens and pencils to a certain degree. However, in printing with an ink jet printer, sufficient printability and drying cannot be obtained, and performance has been unsatisfactory. In printing with an ink jet printer, because a large amount of water is provided on the back surface layer, it is necessary to design the back surface layer taking into consideration water absorption, drying, and coating film strength, as well as printability.

From these viewpoints, there has been proposed a back surface layer having writability by conventional writing instruments and printability in an ink jet printer (see, for example, Japanese Unexamined Patent Publication (Kokai) No. 2001-199172 (page 2), Japanese Unexamined Patent Publication (Kokai) No. 2001-213057 (Page 2), and Japanese Unexamined Patent Publication (Kokai) No. 2003-191652 (page 2)). However, in these back surface layers, general recording is possible by an ink jet printer, but clear image quality cannot necessarily be obtained. Moreover, because the stability of the back surface layer coating material is insufficient and the cost is high, more improvement is required.

Moreover, as the binder for the back surface, a water-soluble resin, such as polyvinyl pyrrolidone is exemplified (see, for example, Japanese Unexamined Patent Publication (Kokai) No. 2000-185476 (pages 7-8)) or Japanese Unexamined Patent Publication (Kokai) No. 2002-337463 (Page 4)). However, when a single-member back surface layer is formed by using a water-soluble resin as a main binder, if printing is performed with an ink jet printer, the drying of the ink is insufficient, and therefore, improvement is required.

## DISCLOSURE OF THE INVENTION

The present invention has been made under these circumstance and provides a receiving sheet having a back surface

layer with good printability by an ink jet printer and sufficient writability for various writing instruments.

The present invention includes the following respective inventions.

- (1) A thermal transfer receiving sheet comprising a sheet-like support, an image receiving layer containing, as a main component, a dye-dyeable resin formed on one surface of the sheet-like support, and a back surface coating layer containing an adhesive resin formed on the other surface of the sheet-like support, wherein the back surface coating layer contains a polyvinyl pyrrolidone resin in an amount of 1 to 50% by weight based on the total solid content of the back surface coating layer.
- (2) The thermal transfer receiving sheet according to (1), wherein a weight average molecular weight of the polyvinyl pyrrolidone resin is from 50,000 to 2,000,000.
- (3) The thermal transfer receiving sheet according to (1) or (2), wherein the back surface coating layer contains an acrylate ester-based resin as the adhesive resin.
- (4) The thermal transfer receiving sheet according to any one of (1) to (3), wherein the back surface coating layer further contains a polyalkylene oxide resin in an amount of 3 to 20% by weight based on the total solid content of the back surface coating layer.
- (5) The thermal transfer receiving sheet according to (4), wherein the polyalkylene oxide resin is a polyethylene oxide resin.
- (6) The thermal transfer receiving sheet according to any one of (1) to (5), wherein the back surface coating layer contains inorganic fine particles and/or organic fine particles.

In the receiving sheet according to the present invention, the back surface layer of the receiving sheet has good printability in an ink jet printer, good adhesiveness for a stamp, and sufficient writability for various writing instruments.

#### BEST MODE FOR CARRYING OUT THE INVENTION

The receiving sheet of the present invention is a receiving sheet having a structure in that the receiving layer for receiving a dye is laminated on one surface of a sheet-like support and the back surface layer is laminated on the surface on which the receiving sheet of the sheet-like support is not formed.

##### (Back Surface Layer)

On the back surface layer of the present invention, a polyvinyl pyrrolidone resin is used in an amount of 1 to 50% by weight based on the total solid content of the back surface layer. The polyvinyl pyrrolidone resin is effective as a material for absorbing water that is the liquid component of the recording media, i.e., ink droplets, or effective as a material for absorbing liquid media for various writing instruments, or further effective as an adhesive resin, or effective for improvement of adhesive strength to the support.

As the adhesive resin used mainly for the back surface layer of the present invention, a conventional adhesive resin can be used and it is also possible to use water-soluble resins such as polyvinyl alcohol resin, polyethylene oxide resin, polyethylene glycol resin, (meta)acrylic acid resin, (meta)acrylate ester resin, starch and the like, and an organic solvent-soluble resin, such as an acrylic resin (e.g. acrylate ester), styrene-butadiene copolymer resin, urethane resin, polyvinyl acetal resin, polyvinyl butyral resin, polyester resin, epoxy resin, melamine resin, phenol resin, phenoxy resin, cellulose derivative resin and the like, and a resin soluble in a mixed solvent composed of water and an organic solvent, such as polyvinyl acetal resin and acrylate resin. These resins may be used singly or two or

more kinds thereof may be used. Moreover, the cured reactants of these resins can be used.

As main components of the adhesive resin for the back surface layer, it is preferable to use an acrylic resin, such as acrylate ester, polyvinyl acetal resin, polyvinyl butyral resin, polyvinyl alcohol resin, starch or phenoxy resin.

It is necessary that the weight ratio of the polyvinyl pyrrolidone resin based on the total solid content of the back surface layer be from 1 to 50% by weight, preferably from 2 to 35% by weight, and more preferably from 3 to 20% by weight. Incidentally, if the weight ratio of the polyvinyl pyrrolidone resin based on the total solid content of the back surface layer is less than 1% by weight, sufficient effect cannot be obtained. On the other hand, if the weight ratio is more than 50% by weight, the waterproof strength of the coating film of the back surface layer tends to decrease.

The polyvinyl pyrrolidone resin of the present invention includes, for example, a homopolymer of a vinyl pyrrolidone, such as N-vinyl-2-pyrrolidone, N-vinyl-4-pyrrolidone, or copolymers of them. Furthermore, the copolymer of vinyl pyrrolidone described above and a copolymerizable monomer can also be used. The copolymerizable monomer other than a vinyl pyrrolidone includes, for example, vinyl monomers such as, styrene, vinyl acetate, (meta)acrylate ester, (meta)acrylonitrile, maleic anhydride, vinyl chloride, vinylidene chloride,  $\alpha$ -olefin, dimethylamino methylmethacrylate, vinylcaprolactam and the like.

Moreover, there can be used a block copolymer or graft copolymer or the like of polyvinyl pyrrolidone and, polyester resin, polycarbonate resin, polyurethane resin, epoxy resin, acetal resin, butyral resin, formal resin, phenoxy resin, cellulose resin, and so forth.

Among these polyvinyl pyrrolidone resins, a homopolymer of vinyl pyrrolidone has good hydrophilicity with an aqueous ink, good coating stability, low cost, and therefore, the homopolymer is preferably used. Moreover, the homopolymer of a vinyl pyrrolidone is preferable because its glass transition temperature is high and the anti-offset property is good. In addition, having the anti-offset property means that when the back surface layer and the printed receiving sheet are superposed, the printed dye of the receiving layer can be prevented from transferring to the back surface layer.

It is preferable that the average molecular weight of the polyvinyl pyrrolidone resin is in a range of 50,000 to 2,000,000, and more preferably 60,000 to 1,800,000. Incidentally, if the weight average molecular weight (Mw) of the polyvinyl pyrrolidone resin is less than 50,000, the adhesiveness between the sheet-like support and the back surface layer may deteriorate, and if the weight average molecular weight is more than 2,000,000, the viscosity of the coating material may rise, resulting in coating property of the back surface layer becoming poor.

If the polyvinyl pyrrolidone resin is used excessively for the back surface layer, although the printability in an ink jet printer and the absorption of an aqueous ink in writing by an aqueous pen would be good, the coating film strength of the back surface layer absorbing an aqueous ink would deteriorate and the back surface layer coating film may deteriorate when contacted with the end of a writing instrument. Therefore, in order to improve ink jet printer printability or coating film strength without writability, it is preferable that as a resin for improving waterproof strength of the coating film, a polyalkylene oxide resin be used together.

As the polyalkylene oxide resin, for example, a polyethylene oxide resin, polypropylene oxide resin, neoxide resin, and so forth are preferably used. Among them, the polyethylene

oxide resin has hydrophilicity, but a low moisture-absorbing property and good affinity with another resin, thereby the waterproof strength of the coating film can be improved, and therefore, the polyethylene oxide resin is more preferably used.

The polyethylene oxide resin used preferably for the back surface layer of the present invention is a resin produced by ring-opening and polymerizing ethylene oxide monomers, and it is preferable that its average molecular weight is in a range of 80,000 to 800,000, more preferably, 100,000 to 500,000. If the average molecular weight is less than 80,000, the effect of improving water-resistance to the coating film is poor, and if the average molecular weight is more than 800,000, there is a possibility that viscosity of the coating material rises, resulting in the coating property of the coating material becoming poor.

It is preferable that a weight ratio of the polyalkylene oxide resin with respect to the total of the solid content weight of the back surface layer is 3 to 20% by weight, more preferably, 4 to 18% by weight. Incidentally, if the weight ratio of the polyalkylene oxide resin with respect to the total of the solid content weight of the back surface layer is less than 3% by weight, the waterproof strength of the coating film of the back surface layer becomes insufficient, and if the weight ratio is more than 20% by weight, the printability of the ink jet printer is in danger of becoming poor.

Acrylate ester-based resins used preferably as the adhesive resin for the back surface layer of the present invention include homopolymers of (meta)acrylate ester or of its derivative, or resins obtained by copolymerizing them and another copolymerizable monomer (such as acrylic acid, methacrylic acid, vinyl acetate, and styrene). Resins can be obtained in the form of an aqueous solution or aqueous dispersion liquid. For this resin coat, a resin coat having water resistance after being dried can be formed and is effective for improving the waterproof strength of the back surface layer coating film.

It is preferable that a weight ratio of the acrylate ester resin with respect to the total of the back surface layer solid content be 3 to 40% by weight, more preferably, 5 to 35% by weight. Incidentally, if the weight ratio of the acrylate ester resin with respect to the total of the back surface layer solid content is less than 3% by weight, the waterproof of the coating film of the back surface layer becomes insufficient, and if the weight ratio is more than 40% by weight, the printability of the ink jet printer may become poor.

It is preferable that the solid content coating amount in the back surface layer be in a range of 0.5 to 10 g/m<sup>2</sup>, and more preferably, 1 to 7 g/m<sup>2</sup>. Incidentally, if the solid content coating amount is less than 0.5 g/m<sup>2</sup>, the back surface layer cannot completely cover the sheet-like support surface, and film defects may arise. On the other hand, if the solid content coating amount is more than 10 g/m<sup>2</sup>, the effect is saturated and the cost becomes higher and is economically disadvantageous.

Furthermore, for the coating solution for forming the back surface layer, optionally various additives such as, an antistatic agent, lubricant, microparticles (also referred to as filler), mold release agent, antifoamer, dispersant, cross-linker for resin, chromatic dye, fluorescent dye, fluorescent pigment, ultraviolet absorber, and so forth may be appropriately selected and used.

In the back surface layer of the present invention, an antistatic agent may be incorporated for preventing paper-feeding or paper-ejecting trouble due to electrostatic charge as well as traveling performance. The antistatic agents include anionic, cationic, nonionic and amphoteric surfactants. Conductive

agents of a high-molecular resin type include a conductive resin of anionic, cationic, and nonionic, inorganic micro powders with electron conductivity, carbon micro powders, and so forth, but the conductive agent of a high-molecular resin type is used preferably because of its long-term antistatic effect and in terms of the hue of the antistatic agent, etc.

As the conductive agent of the high-molecular resin type, a cation-type conductive resin is known to be good, but is expensive and causes amine odor in pyrolysis, and therefore, 10 an anionic conductive resin is preferably used. The anionic conductive resin includes a high molecular containing carboxylic group, sulfonic group, or the like, such as polyacrylic acid, polymethacrylic acid, vinylchloride-maleic acid mono (2-ethylhexyl) copolymer, polystyrene sulfonic acid, and 15 denatured materials thereof, and includes those in which a part or all of the respective functional groups forming alkaline metal salt(s), alkaline earth metal salt(s), or the like. Among them, polyacrylic acid, polymethacrylic acid, and alkali metal salt or alkali earth metal salt of polystyrene sulfonic acid are preferable, and particularly, sodium salt of polystyrene sulfonic acid is preferable because such a salt is excellent in antistatic function, solubility, compatibility with another adhesive resin used together in the back surface layer.

It is preferable that the blending amount of the antistatic agent be 3 to 25% by weight per the total solid content of the back surface layer, and 5 to 20% by weight is further preferable. Incidentally, if the blending amount is less than 3% by weight, surface electric resistance in the receiving sheet back surface side becomes high and sufficient antistatic effect cannot be obtained, and the paper-feeding or paper-ejecting 20 property of the printer, as well as the traveling performance of the receiving sheet may become poor. Moreover, if the blending amount is more than 25% by weight, the strength of the blank sheet coating film of the back surface layer particularly 25 under high temperature and high moisture may deteriorated.

On the back surface layer of the present invention, a lubricant, such as a higher fatty acid salt may be added as the mold release agent. Usable higher fatty acid salts include saturated or unsaturated fatty acid having 12 to 24, preferably, 16 to 20 30 carbons, specifically, lauric acid, myristic acid, palmitinic acid, stearic acid, behenic acid, linoleic acid, oleic acid, and so forth. Preferably, salts of such a higher fatty acid includes metal salt, such as calcium salt, magnesium salt, aluminum salt, zinc salt, and barium salt. Stearic acid metal salt is particularly preferable, and for example, zinc stearate, calcium stearate, barium stearate, and so forth are exemplified.

It is preferable that the blending amount of the lubricant such as the higher fatty acid salt is 3 to 50% by weight based on the total solid content of the back surface layer, and 5 to 40 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 95

surface and is absorbed into the back surface layer, and thereby writing is achieved. Therefore, for achieving good writing properties by pencil and ball-point pen, it is preferable that the back surface layer has appropriate hardness and irregularity.

Moreover, in the back surface layer of the present invention, as the microparticles, inorganic microparticles and/or organic microparticles may be used. The inorganic microparticles include metal such as aluminum, iron, copper, metal oxide such as silica, titanium oxide, zinc oxide, alumina, inorganic salt such as calcium carbonate, barium sulfate, calcium sulfate, and mineral such as kaolin, fired kaolin, clay, talc, diatom earth. Organic microparticles, such as nylon resin, styrene resin, acrylate resin, urea resin, melamine resin, benzoguanamine resin, phenol resin, silicone resin and fluorine resin can be optionally used together. Among these particles, nylon resin particles are preferably used because of appropriately low hardness.

Nylon resin includes resin particles composed of nylon 12, nylon 6, or nylon 6·6. As types of the nylon resin particles, nylon 12 resin particles are preferable because the particles have excellent water resistance and small characteristic change by water absorption, compared to nylon 6 and nylon 6·6 resin particles. It is preferable that the molecular weight of the nylon resin particle be from 100,000 to 1,000,000. A sphere is preferable as its shape, and although its particle diameter cannot be completely determined according to type of the adhesive resin, it is preferable that the size is an average particle diameter of 3 to 30  $\mu\text{m}$ . If the average particle diameter of the nylon resin particles are less than 3  $\mu\text{m}$ , the nylon resin particles are buried in the back surface layer and the friction coefficient lowering effect and the antistatic effect are insufficient, and therefore, the paper-feeding or paper ejecting property, and traveling performance are occasionally bad. On the other hand, if the average particle diameter of the nylon resin particles is greater than 30  $\mu\text{m}$ , the projection of the nylon resin particles from the back surface layer surface becomes significant, and thus when the back surface layer and the receiving layer are strongly contacted with each other, patterns may be made in the receiving layer, thereby a gap may occur in the printing image. Moreover, when the receiving sheet is frictioned, nylon resin particles occasionally drop out. These nylon resin particles may be used singly or two or more kinds may be used together.

It is preferable that the blending amount of the nylon resin particles be 2 to 25% by weight based on the total solid content of the back surface layer, and 3 to 20% by weight is further preferable. Incidentally, if the blending amount is less than 2% by weight, it is difficult to obtain the friction coefficient-lowering effect between the receiving sheets, and the antistatic effect is insufficient, and therefore, overlap feeding of the receiving sheet (which may cause trouble in printing in which a plurality of receiving sheets are fed at the same time in printing of receiving sheet by a printer) may easily occur. On the other hand, if the blending amount is more than 25% by weight, the lines due to precipitation of the nylon resin particles may easily occur, and deterioration of the coating surface may occur. Moreover, the effect for lowering friction coefficient, antistatic efficient, and so forth are saturated and cost increases.

#### (Sheet-Like Support)

As the sheet-like support used in the present invention, there can be exemplified a paper substrate such as coated paper, art paper, and high-quality paper, resin coated paper in which a thermoplastic resin is coated on a paper substrate, laminated paper in which a thermoplastic resin such as polypropylene or polypropylene is extruded and laminated on

a paper substrate, thermoplastic resin film such as polyethylene terephthalate, nylon, polyolefin (such as polypropylene, polyethylene, mixture of polyethylene and polypropylene), film having a structure of a porous monolayer or multilayer in which voids are formed by uniaxially and/or biaxially oriented a melted resin composition in which a thermoplastic resin such as polyolefin resin or polyethylene terephthalate resin and a void-forming agent (inorganic pigment or organic microparticles) serve as main components. Furthermore, not only the above-described material can be used alone, but also a paper having a multilayer structure by bonding two kinds or more of the materials by a known method, such as a dry laminating method, a wet laminating method, or a melting laminating method, and the combination is not limited.

Moreover, on at least one surface of the paper substrate, a coating paper provided with a coating layer containing hollow particles and binders as the main components can also be used.

Also, a sheet-like support composed of an adhesive sheet having a structure of a so-called seal type (also called as sticker or label type) can be used.

It is preferable that a thickness of the sheet-like support be 100 to 300  $\mu\text{m}$ . Incidentally, if the thickness is less than 100  $\mu\text{m}$ , its mechanical strength becomes insufficient and the stiffness of the receiving sheet obtained therefrom and repulsion against deformation becomes insufficient, and curling of the receiving sheet caused during printing cannot be prevented sufficiently. Moreover, if the thickness is more than 300  $\mu\text{m}$ , the thickness of the receiving sheet becomes too great, and this may lead to a problem such as a decrease of the number of the receiving sheets contained in a printer or an increase of the size of the printer. As a result, compactification of the printer may be difficult.

#### (Intermediate Layer)

In the receiving sheet of the present invention, for improvement of adhesiveness between the sheet-like support and the receiving layer, improvement of the antistatic property of the receiving sheet, improvement of barrier property, and so forth, an intermediate layer may be provided. As a resin used for formation of the intermediate layer, various hydrophilic resins or hydrophobic resins can be used, and there can be used, for example, a vinyl polymer such as polyvinyl alcohol and polyvinyl pyrrolidone and its derivative, a polymer containing an acrylic group such as polyacrylic polyacrylamide, polydimethylacrylamide, polyacrylic acid or its salt, and polyacrylate ester, a polymer containing a methacrylic group such as polymethacrylic acid and polymethacrylic ester, and a resin such as polyester-based resin, polyurethane-based resin, starch, denatured starch, and cellulose derivative such as carboxymethyl cellulose. Moreover, known antistatic agents and cross-linking agents can be used singly or used together with the above-described resin(s).

It is preferable that the solid content coating amount of the intermediate layer is in a range of 0.2 to 5  $\text{g}/\text{m}^2$ , further preferably, in a range of 0.5 to 3  $\text{g}/\text{m}^2$ . By the way, if the solid coating amount is less than 0.2  $\text{g}/\text{m}^2$ , the adhesive improving effect is less than the intermediate layer. On the other hand, if more than 5  $\text{g}/\text{m}^2$ , blocking or operating property may deteriorate.

#### (Receiving Layer)

In the receiving sheet of the present invention, the receiving layer provided on one surface of the sheet-like support is formed so that a resin with a dyeing property capable of fixing the dye transferred from the ink ribbon serves as a main component. Such a resin with a dye dyeing property includes

9

polyester resin, vinyl chloride-vinyl acetate copolymer resin, polyvinyl acetal resin, acrylate resin, polycarbonate resin, and cellulose derivative resin.

The solid content coating amount of the receiving layer is controlled in a range of 1 to 12 g/m<sup>2</sup>, preferably, 2 to 10 g/m<sup>2</sup>. Incidentally, if the solid content coating amount is less than 1 g/m<sup>2</sup>, the receiving layer cannot completely cover the support surface, and occasionally, lowering of image quality or the fusing of the receiving layer and the ink ribbon may be caused by heating a thermal head. On the other hand, if the solid content coating amount is 12 g/m<sup>2</sup>, not only the effect is saturated and not economical, but also, the strength of the receiving layer may become insufficient or the insulation effect of the sheet-like support may not be sufficiently exerted and therefore image concentration may become poor.

It is preferable that in the receiving layer, a crosslinking agent, lubricant, and remover for the resin with a dyeing property are added to prevent fusion between the receiving layer and the ink ribbon in thermal heating in a thermal head. Moreover, optionally, another additive such as a chromatic pigment, chromatic dye, fluorescent pigment, fluorescent dye, plasticizer, antioxidant, white pigment, ultraviolet absorber, light stabilizer, and so forth may be added. Such additives may be mixed with the main component of the receiving layer and coated, and may be coated as another coating layer above and/or below the receiving layer.

The coating layers of the receiving sheet of the present invention such as, the intermediate layer, receiving layer, and back surface layer can be formed by being coated and dried by a known coater such as bar coater, gravure coater, comma coater, blade coater, air-knife coater, gate roll coater, dye coater, curtain coater, and slide bead coater, and so forth.

## EXAMPLES

The present invention will now be described in detail with reference to the following Examples and Comparative Examples, but the scope of the present invention is not limited thereto. In the Examples and Comparative Examples, parts and percentages are by weight unless otherwise specified.

The molecular weight of the polyvinyl pyrrolidone used herein was analyzed by using a column for analyzing gel permeation chromatography (GPC) (trade name: Showdex SB-805 HQ, manufactured by Showa Denko Co., Ltd.) and using a mixture of an aqueous NaNO<sub>3</sub> solution and acetonitrile in a weight ratio of 90:10 as the solvent. As a standard sample, commercially available polyvinyl pyrrolidone (manufactured by Wako Pure Chemical Industries, Ltd) having a known molecular weight was used.

The molecular weight of the polyethylene oxide used herein was analyzed by using a column for analyzing gel permeation chromatography (GPC) (trade name: Showdex asahipak CF-710 HQ, manufactured by Showa Denko Co., Ltd.) and using LiCl (having a concentration of 50 mM) as the solvent. As a standard sample, TSK polyethylene oxide (manufactured by Tosoh Co., Ltd.) having a known molecular weight was used.

### Example 1

On the front and back surfaces of a polyethylene terephthalate (PET) film having a thickness of 50 µm, a biaxially oriented porous multilayered film (trade name: YUPO FPG60, manufactured by YUPO Corporation) having a thickness of 60 µm, which contains an inorganic pigment and

10

contains polyolefin as a main component, was laminated using a polyester-based adhesive to obtain a sheet-like support.

On one surface of the support, the following coating solution for receiving layer-1 was coated using a gravure coater and then dried to form a receiving layer having a coating amount (solid content) of 5 g/m<sup>2</sup>. Then, the receiving layer was crosslinked by maintaining in an atmosphere of 50° C. for 3 days.

#### Coating solution for receiving layer-1

|    |                                                                                                       |           |
|----|-------------------------------------------------------------------------------------------------------|-----------|
| 15 | Polyester resin<br>(trade name: Byron 200, manufactured by Toyobo Co., Ltd.)                          | 100 parts |
|    | Silicone oil<br>(trade name: KF393, manufactured by Shin-Etsu Chemical Co., Ltd.)                     | 3 parts   |
| 20 | Isocyanate compound<br>(trade name: Takenate D110N, manufactured by Mitsui Takeda Chemical Co., Ltd.) | 5 parts   |
|    | Mixed solution of toluene and methyl ethyl ketone in a weight ratio of 1:1                            | 400 parts |

On the surface opposite to the surface on which the receiving layer was formed, of the sheet-like support, the following coating solution for back surface layer-2 was coated using a gravure coater and then dried to obtain a back surface later having a coating amount (solid content) of 3 g/m<sup>2</sup>.

#### Coating solution for back surface layer-2

|    |                                                                                                                                                             |           |
|----|-------------------------------------------------------------------------------------------------------------------------------------------------------------|-----------|
| 35 | Polyvinyl pyrrolidone resin<br>(trade name: Polyvinyl pyrrolidone K90, weight average molecular weight: 1,600,000, manufactured by ISP Japan Co., Ltd.)     | 45 parts  |
| 40 | Acrylate ester resin<br>(trade name: Julimar AT613, manufactured by Nihonjyunaku Co., Ltd.)                                                                 | 15 parts  |
|    | Nylon resin particle<br>(trade name: MW330, nylon 12 resin, average particle diameter: 7 µm, manufactured by Shinto Paint Co., Ltd.)                        | 10 parts  |
| 45 | Zinc stearate<br>(trade name: KW509, manufactured by Goo Chemical Co., Ltd.)                                                                                | 20 parts  |
|    | Anionic conductive resin<br>(trade name: CHEMISTAT SA-9, main component: sodium polystyrene sulfonate, manufactured by Sanyo Chemical Industries Co., Ltd.) | 10 parts  |
| 50 | Mixed solution of water and isopropyl alcohol in a weight ratio of 2/3                                                                                      | 500 parts |

### Example 2

55 In the same manner as in Example 1, except that the amount of the polyvinyl pyrrolidone resin was replaced by 30 parts and the amount of an acrylate ester resin was replaced by 30 parts in the coating solution for back surface layer-2 of Example 1, a receiving sheet was obtained.

### Example 3

65 In the same manner as in Example 1, except that the following coating solution for back surface layer-3 was used instead of the coating solution for back surface layer-2, a receiving sheet was obtained.

| Coating solution for back surface layer-3                                                                                                                   |           |    |
|-------------------------------------------------------------------------------------------------------------------------------------------------------------|-----------|----|
| Polyvinyl pyrrolidone resin<br>(trade name: Polyvinylpyrrolidone K90, weight average molecular weight: 1,600,000, manufactured by ISP Japan Co., Ltd.)      | 18 parts  | 5  |
| Acrylate ester resin<br>(trade name: Julimar AT613, manufactured by Nihonjyunaku Co., Ltd.)                                                                 | 27 parts  |    |
| Nylon resin particle<br>(trade name: MW330, nylon 12 resin, average particle diameter: 7 $\mu\text{m}$ , manufactured by Shinto Paint Co., Ltd.)            | 15 parts  | 10 |
| Zinc stearate<br>(trade name: KW509, manufactured by Goo Chemical Co., Ltd.)                                                                                | 25 parts  |    |
| Anionic conductive resin<br>(trade name: CHEMISTAT SA-9, main component: sodium polystyrene sulfonate, manufactured by Sanyo Chemical Industries Co., Ltd.) | 15 parts  | 15 |
| Mixed solution of water and isopropyl alcohol in a weight ratio of 2/3                                                                                      | 500 parts |    |

## Example 4

In the same manner as in Example 1, except that the amount of the polyvinyl pyrrolidone resin K90 was replaced by 5 parts in the coating solution for back surface layer-3 of Example 3, a receiving sheet was obtained.

## Example 5

In the same manner as in Example 3, except that a polyvinyl pyrrolidone resin (trade name: polyvinyl pyrrolidone resin K30, weight average molecular weight was 70,000, manufactured by ISP Japan Co., Ltd.) was used instead of a polyvinyl pyrrolidone resin K90 in the coating solution for back surface layer-3 of Example 3, a receiving sheet was obtained.

## Example 6

In the same manner as in Example 1, except that the following coating solution for back surface layer-4 was used instead of the coating solution for back surface layer-2 in Example 1, a receiving sheet was obtained.

| Coating solution for back surface layer-4                                                                                                                   |           |   |
|-------------------------------------------------------------------------------------------------------------------------------------------------------------|-----------|---|
| Polyvinyl pyrrolidone resin<br>(trade name: Polyvinyl pyrrolidone K90, weight average molecular weight: 1,600,000, manufactured by ISP Japan Co., Ltd.)     | 11 parts  | 5 |
| Polyethylene oxide resin<br>(trade name: ALKOXOR150, weight average molecular weight: 140,000, manufactured by Meisei Chemical Works, Ltd.)                 | 11 parts  |   |
| Acrylate ester resin<br>(trade name: Julimar AT613, manufactured by Nihonjyunaku Co., Ltd.)                                                                 | 27 parts  |   |
| Nylon resin particle<br>(trade name: MW330, nylon 12 resin, average particle diameter: 7 $\mu\text{m}$ , manufactured by Shinto Paint Co., Ltd.)            | 15 parts  |   |
| Zinc stearate<br>(trade name: KW509, manufactured by Goo Chemical Co., Ltd.)                                                                                | 25 parts  |   |
| Anionic conductive resin<br>(trade name: CHEMISTAT SA-9, main component: Sodium polystyrene sulfonate, manufactured by Sanyo Chemical Industries Co., Ltd.) | 15 parts  |   |
| Mixed solution of water and isopropyl alcohol in a weight ratio of 2/3                                                                                      | 500 parts |   |

## Example 7

In the same manner as in Example 6, except that the amount of a polyvinyl pyrrolidone resin was replaced by 6 parts and the amount of a polyethylene oxide resin was replaced by 6 parts in the coating solution for back surface layer-4 of Example 6, a receiving sheet was obtained.

## Comparative Example 1

In the same manner as in Example 1, except that the back surface layer was not formed in Example 1, a receiving sheet was obtained.

## Comparative Example 2

In the same manner as in Example 1, except that a polyvinyl alcohol resin (trade name: PVA105, manufactured by Kuraray Co., Ltd.) was used in place of the polyvinyl pyrrolidone resin, a receiving sheet was obtained.

## Comparative Example 3

In the same manner as in Example 1, except that the amount of the polyvinyl pyrrolidone resin was replaced by 55 parts and the amount of the acrylate ester resin was replaced by 5 parts in the coating solution for back surface layer-2 of Example 1, a receiving sheet was obtained.

## Quality Evaluation

The receiving sheets obtained in Examples 1 to 7 and Comparative Examples 1 to 3 were subjected to the following quality evaluation tests. The evaluation results are shown in Table 1.

## [Ink Jet Printer Compatibility]

The receiving sheet was set in an ink jet printer (trademark: BJC610JW, manufactured by Canon Co., Ltd.), and the letter image was printed on the surface of a back surface layer of the ink jet sheet at a mode of 720 dpi  $\times$  720 dpi, and printability using the ink jet printer was evaluated by the following criteria.

Excellent: Blur of the letter does not occur at all and the letter is easy to read; excellent printability

Good: slight blur occurs but is readable with no problems; good printability

Fair: slight blur of the letter occurs, but it is possible to put into practical use

Failure: severe blur of the letter occurs and cannot be read; it is impossible to put into practical use

## [Printing Water Resistance of Ink Jet Printer]

The receiving sheet was set in an ink jet printer (trademark: BJC610JW, manufactured by Canon Co., Ltd.), and the letter image was printed on the surface of a back surface layer surface of the ink jet sheet at a mode of 720 dpi  $\times$  720 dpi mode. After dropping one water droplet on the printed area and slightly rubbing with tissue paper, water resistance of the printed image was evaluated by the following criteria.

Excellent: Image is not removed when the printed surface is rubbed; excellent water resistance

Good: Image is slightly removed when the printed surface is rubbed; good water resistance

Fair: Image is slightly removed when the printed surface is rubbed; it is possible to put in practical use

Failure: Image is severely removed when the printed surface is rubbed; it is impossible to put in practical use

## [Stamp Adhesion Property]

The entire surface of an adhesive surface of Japanese 50-yen postal stamp was coated with tap water using fingers

## 13

and the stamp was applied onto the back surface layer surface of the receiving sheet. The stamp was allowed to stand for 24 hours, and then the stamp adhesion was evaluated by the following criteria.

Good: Stamp adheres after 24 hours

Failure: Stamp does not adhere after 24 hours and can be peeled off by hand after 24 hours; it is impossible to put into practical use.

## [Writability]

As writing utensils used generally, a pencil (hardness HP), a ball pen, an aqueous pen and an oily pen were prepared, and a letter was written on the surface of a back surface layer surface of a receiving sheet, and then writability was generally evaluated by the following criteria.

Excellent: Any blur of the letter does not occur at all; good writability

Good: Slight blur of the letter occurs in case of some writing utensils; good writability

Fair: Slight blur of the letter occurs in case of some writing utensils; it is possible to put into practical use

Failure: Severe blur of the letter occurs; it is impossible to read, write and put into practical use

TABLE 1

|                       | Ink jet printer compatibility |                           | Stamp             |             |
|-----------------------|-------------------------------|---------------------------|-------------------|-------------|
|                       | Printability                  | Printing water resistance | adhesion property | Writability |
| Example 1             | Fair                          | Fair                      | Good              | Fair        |
| Example 2             | Good                          | Good                      | Good              | Fair        |
| Example 3             | Excellent                     | Good                      | Good              | Good        |
| Example 4             | Good                          | Excellent                 | Good              | Good        |
| Example 5             | Good                          | Good                      | Good              | Good        |
| Example 6             | Excellent                     | Excellent                 | Good              | Excellent   |
| Example 7             | Excellent                     | Excellent                 | Good              | Excellent   |
| Comparative Example 1 | Failure                       | Failure                   | Failure           | Failure     |
| Comparative Example 2 | Failure                       | Failure                   | Good              | Fair        |
| Comparative Example 3 | Failure                       | Failure                   | Good              | Fair        |

40

## 14

## INDUSTRIAL APPLICABILITY

In the receiving sheet of the present invention, the back surface layer has good printability by an ink jet printer and also has sufficient writability for various writing instruments, and therefore the receiving sheet can be utilized as a receiving sheet which is inexpensive and has high practical value.

10 The invention claimed is:

1. A thermal transfer receiving sheet comprising a support, an image receiving layer containing, as a main component, a dye-dyeable resin formed on one surface of the support, and a back surface coating layer containing an adhesive resin formed on the other surface of the sheet-like support, wherein the back surface coating layer further contains a polyvinyl pyrrolidone resin and a polyalkylene oxide resin,

wherein the polyvinyl pyrrolidone resin is in an amount of

1 to 50% by weight based on the total solid content of the back surface coating layer and wherein the weight ratio of the polyalkylene oxide resin with respect to the total of the solid content weight of the back surface layer is 3 to 20% by weight.

20 2. The thermal transfer receiving sheet according to claim 1, wherein a weight average molecular weight of the polyvinyl pyrrolidone resin is from 50,000 to 2,000,000.

25 3. The thermal transfer receiving sheet according to claim 1 or 2, wherein the back surface coating layer contains an acrylate ester-based resin as the adhesive resin.

30 4. The thermal transfer receiving sheet according to claim 1 or 2, wherein the back surface coating layer contains inorganic fine particles and/or organic fine particles.

35 5. The thermal transfer receiving sheet according to claim 1, wherein the polyalkylene oxide resin is a polyethylene oxide resin.

\* \* \* \* \*